

## UNITED STATES PATENT OFFICE

2,279,499

PROCESS OF COMBINING HARDENABLE  
PHENOL - ALDEHYDE CONDENSATION  
PRODUCTS WITH AIR-DRYING FATTY  
OILSFritz Seebach, Erkner, near Berlin, Germany,  
assignor, by mesne assignments, to Bakelite  
Corporation, a corporation of New JerseyNo Drawing. Application February 12, 1930,  
Serial No. 427,993. In Germany February 25,  
1929

6 Claims. (Cl. 260—19)

Resoles, i. e. synthetic resinous products of a hardenable nature in their fusible and soluble initial condition, and air-drying, fatty oils cannot be mixed or are insoluble in each other. This constitutes a serious disadvantage, for resoles otherwise have properties that are valuable in oil varnishes. Accordingly there has been no lack of experimentation to render resoles oil-soluble; but in all processes heretofore made known the character of the resoles is considerably changed in imparting the oil-soluble property thereto. The obtained products show a novolak character, that is, they remain fusible and soluble under the application of heat, and they can as a result be combined with oils at the usual high temperatures employed in the lacquer or varnish practice. However, if the resole character is to be retained such methods of working are out of the question on account of the readily initiated conversion of the resoles to their infusible and insoluble condition which takes place under application of heat. It has been proposed to simply mix a resole with an air-drying oil in a common solvent at temperatures which do not cause transformation of the resole. As a matter of fact such solutions are readily obtained; but a separation of oil and resole takes place to a degree corresponding to the evaporation of the solvent either from a coating made with the solution or from the solution.

We have now found that air-drying oils which are in some manner combined with more or less oxygen show an entirely different behavior towards resoles. Air-drying fatty oils, for example, which contain a small proportion of their own oxidation products in solution, or which have undergone a mild oxidation throughout their mass, may be incorporated with resoles in any proportion and used in lacquers to yield surfaces that remain glossy. The composite oil and resole products have the surprising property of solution in or dilution with solvents that are otherwise non-solvents for one of the two components, either the oil or the resole. For instance, a varnish made with such products can be diluted with turpentine alone or with wood alcohol alone. Films deposited therefrom are hardenable to an exceptional degree. They are resistant to mechanical and chemical influences; as an instance they are not changed when subjected for days to the action of organic solvents such as benzene, alcohol, etc.

Resoles for incorporation with air-drying oils according to this invention can be produced in any suitable manner, for example, by the condensation of phenol or cresol with an aldehyde

such as formaldehyde, using ammonia as a condensing agent. Resoles made by the addition of hardening agents to novolaks can be used, or a mixture of several resoles. Suitable air-drying 5 oils are linseed oils, China wood oil, perilla oil, poppyseed oil, linseed-stand oil or mixtures of these oils. Oxidation of these oils can be accomplished in the usual manner, for example, by the action of air at ordinary or elevated temperatures, simple exposure to the air, short-wave rays, ozonization, etc. Several air-drying oils can be mixed together and then oxidized or the oils can be separately oxidized and then mixed.

The oxidation of the oils can be carried out in 15 the presence of the resoles by distributing the resoles in the fatty oils as a suspension or by means of a solvent.

The association of air-drying fatty oils with resoles becomes easier with increased oxidation 20 of the air-drying fatty oil. No treatment of any kind is required, for example, if an alcohol solution of the resole is mixed with a solution of linoxin in any solvent, for instance, cyclohexanol, or a suitable solvent mixture at ordinary temperatures. Coatings obtained with such oil varnishes remain glossy under all conditions, whether they be air dried or hardened by heat at elevated temperatures, and therefore exceptionally desirable. A similar mixture in solution 25 containing linseed oil varnish instead of linoxin would upon air drying as well in hardening by heat become turbid and therefore not usable. With the use of air-drying fatty oils which are oxidized to but a small percentage of their oxygen absorbing capacity it is generally not sufficient to mix resoles with them in any kind of solvent at ordinary temperatures; in such cases both components should be heated for some time and preferably in the presence of a diluting agent. The heating temperature and the heating 30 period may be decreased in proportion to the increased absorption of oxygen by the air-drying oil. The combination of air-drying fatty oils with resoles can be hastened by the presence of certain catalysts, such as lead oxide. Catalysts are especially desirable if the air-drying oils contain but a small amount of oxidation products. For example, resoles can be combined with linseed oil or the like by boiling the oil with a solution of the resole in the presence of oxygen bearing catalysts, such as lead oxide, manganese oxide, etc., or combinations of these substances with fatty oils or resins. Several catalysts can be used in admixture or two or more of them 35 used consecutively. The quantity of catalyst to be added varies with the different oils. With linseed oils, for example, more catalyst is re-

quired than with China wood oils; in the latter case extremely small traces are enough and one can even do without the catalyst if the reaction temperature is maintained longer than usual. The presence of catalysts hastens the process.

By the procedure here described products are obtained from linseed oil or linseed oil solutions and hardenable resins which yield a clear drying film that can be dried either in air or at elevated temperatures.

*Example 1*

1 part by weight of a resole prepared by condensation.

1 part by weight of an air-blown linseed oil.  
1 part by weight of a solvent dissolving both substances equally well, for example, cyclohexanol or a 1:1 mixture of turpentine and wood alcohol or a 1:1 mixture of benzol-wood alcohol.

are heated for  $\frac{1}{4}$  or  $\frac{1}{2}$  hour at 80–100° C. Then the volatile ingredients are removed under a vacuum while the temperature should not exceed 100°. After removal of the volatile ingredients a substance is obtained that is extremely tough at room temperature, yet perfectly clear, consisting of about equal proportions of resole and fatty oil. The product in this consistency is similar to softer kinds of resoles and in appearance is hardly to be distinguished from them. The clear solubility of the product in wood alcohol or in oil of turpentine is remarkable. The films obtained from such solutions quickly dry in the air and after hardening on metal yield elastic coatings resistant to organic solvents, such as carbon disulfide.

*Example 2*

The procedure is the same as in Example 1, however, instead of air-blown linseed oil a mixture of equal portions of ordinary China wood oil and air-blown linseed oil are applied. The finished product is clearly soluble in oil of turpentine or in an oil of turpentine-wood alcohol mixture and it yields clear drying and clear hardening films.

*Example 3*

Parts  
Resole prepared from technical cresol by condensation with formaldehyde and ammonia. 50  
Solvents as per Example 1. 50  
Stand-oil of air-blown linseed oil. 12

are heated to 100° C. for 1½ hours or  $\frac{1}{2}$  hour to 160° if desired under pressure, and the solvent is driven off under a vacuum. The finished product is soluble in wood alcohol or in a mixture of wood alcohol and turpentine.

*Example 4*

Parts  
Hardenable condensation products from cresol, formaldehyde and ammonia. 75  
Solvents as per Example 1. 150  
Linseed oil varnish. 75  
Lead oxide or 3 parts manganese oxide. 6

are heated to 120° C. for 1 hour, if desired under pressure. Then the volatile solvent is driven off under a vacuum. The residue is bright and easily soluble in a turpentine-wood alcohol mixture. In the oils, which as specified in the example, are to be combined with the resoles one may dissolve other resins also, as for example, natural resins or synthetic resins and proceed

analogous to the above examples. One may however dissolve in the oils such substances also that ordinarily do not combine with hardenable phenol condensation products, as for example, caoutchouc.

*Example 5*

|                                                                                                                                                                                                                                                                                                                                                                                                                                                                                                                                                                                                                                                                                                                                                                                                                                                                                          | Parts by weight |
|------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-----------------|
| Hardenable phenol-aldehyde condensation products                                                                                                                                                                                                                                                                                                                                                                                                                                                                                                                                                                                                                                                                                                                                                                                                                                         | 2               |
| 10 Melt of oxidized linseed oil and caoutchouc in the proportion of 1:1                                                                                                                                                                                                                                                                                                                                                                                                                                                                                                                                                                                                                                                                                                                                                                                                                  | 2               |
| 15 Solvents according to Example 1                                                                                                                                                                                                                                                                                                                                                                                                                                                                                                                                                                                                                                                                                                                                                                                                                                                       | 4               |
| are heated together at a temperature of 100–130° C. until the fusion is completed. The films thus produced are bright. The varnishes or films may be vulcanized.                                                                                                                                                                                                                                                                                                                                                                                                                                                                                                                                                                                                                                                                                                                         |                 |
| 20 One may also obtain molded parts from the combination products of hardenable phenol-aldehyde condensation products and air-drying oils by charging the molds with the heated product if desired after admixture with fillers, dyes or other suitable additions and by hardening for example at temperatures of 80–150° C. Perfectly clear, hard, elastic substances can thus be obtained. The products obtained according to the invention may furthermore be used for impregnation. Superposed layers of paper, that is, for example, saturated with a wood alcohol solution of the described combination products from resoles and air-drying oils may be molded under heat and pressure into solid pieces. Instead of a single solvent one may in this instance as in all the others use suitable solvent mixtures in the preparation and application of the combination products. |                 |

I claim:

1. Process of preparing compositions which comprises mixing a hardenable phenol-aldehyde condensation product with an oxidized air-drying fatty oil in a solvent for both components and thereafter removing the solvent.

2. Process of preparing compositions which comprises mixing a hardenable phenol-aldehyde condensation product with an oxidized air-drying fatty oil in a solvent for both components and thereafter removing the solvent under reduced pressure.

3. In a process of preparing compositions from hardenable phenol-aldehyde condensation products and air-drying fatty oils the step which comprises oxidizing an air-drying fatty oil in the presence of the hardenable phenol-aldehyde condensation product.

4. In a process of preparing compositions from hardenable phenol-aldehyde condensation products and air-drying fatty oils the step which comprises oxidizing an air-drying fatty oil in the presence of the hardenable phenol-aldehyde condensation product, said condensation product being distributed as a suspension in the oil.

5. Process of preparing compositions which comprises mixing hardenable phenol-aldehyde condensation product with an oxidized air-drying fatty oil in a solvent for both components and with the application of heat, and thereafter removing the solvent.

6. Process of preparing compositions which comprises mixing a hardenable phenol-aldehyde condensation product with an oxidized air-drying fatty oil in a solvent for both components and with the application of heat, and thereafter removing the solvent under reduced pressure.

CERTIFICATE OF CORRECTION.

Patent No. 2,279,499.

April 14, 1942.

FRITZ SEEBACH.

It is hereby certified that error appears in the printed specification of the above numbered patent requiring correction as follows: Page 2, second column, line 69, claim 6, for "pheno-aldehyde" read --phenol-aldehyde--; and that the said Letters Patent should be read with this correction therein that the same may conform to the record of the case in the Patent Office.

Signed and sealed this 16th day of June, A. D. 1942.

(Seal)

Henry Van Arsdale,  
Acting Commissioner of Patents.